

## UNITED STATES PATENT OFFICE

2,391,653

## GOLDBEATER LUBRICATION MATERIAL

Donald D. Swift, Hartford, Conn., assignor to  
M. Swift & Sons, Inc., a corporation of Con-  
necticut

No Drawing. Original application October 28,  
1939, Serial No. 301,797, now Patent No.  
2,354,072, dated July 18, 1944. Divided and this  
application July 18, 1944, Serial No. 545,539

2 Claims. (Cl. 252—42.1)

This application is a division of application  
Serial No. 301,797, filed October 28, 1939, Gold-  
beating lubricant, now Patent No. 2,354,072, pat-  
ented July 18, 1944.

My present invention relates to the goldbeater's  
art and more particularly to an improved lubri-  
cant to be used with goldbeater's skin.

In beating gold or other metallic leaf, it is  
customary to place small squares of gold in a  
packet, each square between sheets of cutch pa-  
per, the entire packet then being beaten until the  
gold or other metal spreads to the size of the  
enclosing sheets. The metal is then quartered  
and the quarters are placed between packets of  
goldbeater's skin and further beaten. This proc-  
ess is continued until the leaf has reached the  
desired size and thinness.

The conventional goldbeater's skins are of ani-  
mal origin, but substitutes such as Cellophane or  
cellulose acetate may be used. To facilitate the  
beating operation, it is customary to "doctor" the  
goldbeater's skin or the substitute and to add a  
suitable lubricant. The conventional doctoring  
long used for this purpose consists essentially of  
isinglass, gum arabic, shellac, and spices such as  
saffron, cinnamon, and cloves in red wine. The  
lubricant is usually made up from soap, gypsum,  
and water, or in some instances, alcohol.

I have found that a greatly improved gold-  
beater's lubricant is obtained by the use of a  
mineral carrier which is soft enough to be  
scratched by a fingernail and which can be sub-  
divided to almost microscopic dimensions. I have  
found that the imbedding of such a mineral car-  
rier in a fatty acid sodium salt produces a far  
superior lubricant.

To this end, I prepare the lubricant of the pres-  
ent invention by dissolving a fatty acid sodium  
salt such as sodium stearate or sodium palmitate  
in a suitable alcohol such as propyl alcohol; suit-  
able organic soaps may be used in place of the  
sodium stearate or palmitate. The desired char-  
acteristics of the salt are that it be soluble in al-  
cohol, non-adhesive, with a fairly high melting  
point and chemically stable. A mineral carrier  
meeting the aforementioned requirements, such  
as completely dehydrated calcium sulphate, in

powder form, is then mixed into the solution; an  
alkaline earth soap, such as calcium, magnesium  
or zinc stearate, may be used instead of the cal-  
cium sulphate. It is preferred that a uniform  
mixture be obtained so that the fine particles  
of the dehydrated calcium sulphate powder or  
soap are suspended in the solution of the sodium  
stearate or sodium palmitate in alcohol, the alco-  
hol tending to inhibit hydrolysis of the soap. The  
alcohol is then evaporated by any suitable, well-  
known method and the residue is a smooth, fine-  
grained lubricant far superior to any that have  
heretofore been used.

It is preferred to use such proportions of the  
sodium stearate or sodium palmitate and the  
completely dehydrated calcium sulphate that the  
final product comprises particles of calcium sul-  
phate each covered with a surface layer of soap.  
For example, 6½ oz. of sodium stearate are dis-  
solved in about 3 qts. of alcohol. After the soap  
is completely dissolved, 12 lbs. of completely de-  
hydrated calcium sulphate in a finely powdered  
form are slowly stirred into the solution. The  
alcohol is then evaporated.

The resultant lubricant is fine grained, soft,  
will not scratch or puncture the gold or other  
metallic leaf during the beating operation and  
has very superior lubricating qualities.

While I have described a specific mineral car-  
rier and specific soaps, it is obvious that other  
carriers and other soaps or their equivalents may  
be used in varying proportions, without departing  
from the spirit and the scope of the invention  
as defined in the appended claims.

I claim:

1. The method of preparing a lubricant for  
metal beating, comprising the steps of dissolving  
sodium palmitate in alcohol, mixing completely  
dehydrated calcium sulphate uniformly therein  
to obtain a suspension of the calcium sulphate  
in the solution of sodium palmitate, and evap-  
orating the alcohol.

2. An improved lubricant for metal beating  
comprising comminuted particles of dehydrated  
calcium sulphate, each particle being covered by  
a surface layer of sodium palmitate.

DONALD D. SWIFT.